

# UNITED STATES PATENT OFFICE.

AUGUST LEUCHTER, OF NEW YORK, N. Y.

## ELECTROPLATING.

1,026,628.

No Drawing.

Specification of Letters Patent.

Patented May 14, 1912.

Application filed February 15, 1912. Serial No. 677,869.

*To all whom it may concern:*

Be it known that I, AUGUST LEUCHTER, a citizen of the United States, residing at New York, borough of Brooklyn, county of Kings, and State of New York, have invented certain new and useful Improvements in Electroplating, of which the following is a full, clear, and exact description.

10 By the invention which forms the subject of my present application, and which is an improvement in the art of electro-plating, I am enabled to produce an electrolytically deposited surface which is lustrous and of 15 more pleasing appearance than nickel; extremely hard and durable, and, under all ordinary conditions of use, non-corrosive.

The improvement involves the electro-coating or plating of articles with nickel 20 and manganese, in what appears to be an alloy of these two metals, and is effected in the following manner: In an apparatus of the kind usually employed in the operation of electro-plating with silver or nickel, I 25 use an anode composed essentially of nickel and manganese to which has been added a sufficient proportion of tin to make an alloy, but in which the nickel very largely predominates, constituting, preferably 98 per 30 cent. of the whole. This anode is used in a bath composed of or containing nickel ammonium sulfate and manganese ammonium sulfate, the nickel predominating, being preferably present in the proportion of 35 85 per cent. to 15 per cent. of manganese. By means of this bath, articles of iron, steel, brass or other metals of not too soft or coarse a texture may be coated in the ordinary way, with a surface greatly superior to 40 any other of which I am aware in the respects noted above. If it be desired to increase the hardness of the deposited surface a small proportion of chromium, in solution may be added to the electrolyte.

Beyond the requirement that in the anode 45 the nickel should very largely predominate, and that in the electrolyte there should be present a much larger percentage of nickel, the proportions of the several ingredients of the anode and the bath may be varied to 50 a considerable extent, the permissible limits for good results being dependent upon readily recognized conditions in actual use. For example the anode may contain as much as 55 seven per cent. of manganese and the proportion of this metal in the bath may be as high as twenty five per cent. I have found, however, that the best results are secured by substantially the proportions first above stated.

What I claim is:

1. An electro-plating bath comprising an anode of nickel and manganese, and an electrolyte containing the salts of nickel and of manganese.

2. An electro-plating bath comprising an anode of nickel and manganese alloy and an electrolyte containing the salts of nickel and of manganese.

3. An electro-plating bath comprising an 70 anode of nickel and manganese in which the nickel predominates, and an electrolyte containing nickel and manganese, the nickel predominating.

4. An electro-plating bath comprising an 75 anode of nickel alloyed with from two to seven per cent. of manganese, and a bath containing nickel ammonium sulfate and manganese ammonium sulfate the nickel being present in the proportions of from 80 75 to 85 per cent. to from 25 to 15 per cent. of manganese.

In testimony whereof I affix my signature in the presence of two subscribing witnesses.

AUGUST LEUCHTER.

Witnesses:

M. LAWSON DYER,  
B. R. SANDMAN.